

April 18, 1933.

K. WINKLER ET AL

1,904,586

CONVERSION OF CARBONACEOUS SOLIDS INTO VALUABLE LIQUID PRODUCTS

Filed Dec. 15, 1927



INVENTORS  
Karl Winkler  
BY Kurt Wissel  
Hennig-Brandt  
ATTORNEYS

## UNITED STATES PATENT OFFICE

KARL WINKLER AND KURT WISSEL, OF LUDWIGSHAFEN-ON-THE-RHINE, GERMANY,  
ASSIGNEES TO I. G. FARBENINDUSTRIE AKTIENGESELLSCHAFT, OF FRANKFORT-  
ON-THE-MAIN, GERMANY, A CORPORATION OF GERMANY

## CONVERSION OF CARBONACEOUS SOLIDS INTO VALUABLE LIQUID PRODUCTS

Application filed December 15, 1927, Serial No. 240,333, and in Germany December 22, 1928.

In the process of low temperature carbonization of solid bituminous materials a large proportion of the said materials is converted into difficultly condensable gases at the expense of the yield of tar.

We have now found that an excellent yield of liquid products and of products which liquefy when warm i. e. at temperatures not much above ordinary temperature are obtained, and the formation of gases, and especially such gases as condense with difficulty, is prevented to a large extent, by treating the solid initial materials in the absence of substantial amounts of added hydrogen with high boiling hydrocarbons or hydrocarbons having a high molecular weight, which expression is also understood to comprise the derivatives thereof, containing substantially no constituents boiling below 300° C., in a suitable pressure chamber, if desired with the joint use of gases containing for example nitrogen, carbon dioxid or carbon monoxid but free from considerable amounts of hydrogen, and/or the joint addition of catalytic substances, such for example as substances with alkaline reaction, in particular the sulfids of the alkali metals and alkaline earth metals, at temperatures below the coking temperature of the added hydrocarbons or their derivatives, in a continuous manner and under elevated pressure, preferably very high pressure, for such a period of time that the yield of valuable hydrocarbons or hydrocarbon derivatives becomes a multiple of that obtained by ordinary low temperature carbonization. By continuous treatment is meant the continuous introduction of the materials to be treated and the continuous removal of the products of the process.

The employment of inert gases is particularly advantageous since these loosen up the material under treatment and since they may also increase the pressure on the material and since on account of their diluent action they

allow of a more rapid running through of the materials.

The addition of the aforesaid catalytic substances has the great advantage that the products extracted by the solvent are considerably improved. For example unsaturated compounds may be polymerized and on the other hand a too far reaching condensation of these compounds with the formation of resinous substances, which may obstruct the speed of the extracting operation and the yields obtained therein, is prevented. In this manner the said catalysts indirectly increase the speed of the operation and the resulting yields. The amounts of catalyst used are not critical for the improved result. Improved results are obtained even with very small amounts of catalyst, and amounts considerably larger than those required for securing a desired degree of improvement have no detrimental effect. In practice the catalyst is employed in an amount of about from 3 to 7 per cent of the weight of the mixture of coal and oil treated. A great variety of solid bituminous initial materials may be employed according to the new process, as for example different kinds of coal, such as pit coal or brown-coal of varied origin and character, even that which has already been deprived of bitumen by extraction, as well as bituminous shales, peat, wood and the like.

The added oils comprise high-boiling hydrocarbons or hydrocarbons of high molecular weight, or their derivatives, of the most varied origin and nature. Suitable materials are for example liquid hydrocarbons or their derivatives or those liquefying when warm, which are substantially free from constituents boiling below 300° C. and which are obtained from any varieties of coal, tars, mineral oils and the like, their distillation and conversion product and residues, as for example by cracking, destructive hydrogenation and other like methods. Use

may also be made, for example, of high boiling products such as are prepared synthetically from hydrogen and oxids of carbon and the like, and of course the products obtained in the process of the present invention itself may also be employed. Moreover, oils of different kinds may be employed in succession or in association.

In addition to the high-molecular added oils, use may be made of gases such as nitrogen, ammonia, carbon dioxide, water vapor, and the like. At the temperatures and pressures employed according to the present invention no substantial dissociation of ammonia or water into their elements occurs, so that substantially no hydrogenation takes place. Other additions may also be made which have a beneficial physical or chemical action, such as distributive, thermoconductive or catalytic action, during the process.

The temperature must be regulated according to the substance employed and may vary for different materials. Elevated temperatures may be employed without however exceeding the coking temperature of the added oils under the specified working conditions. In many instances, the most favorable working temperature may be about 300° C. but higher and lower temperatures may also be employed, a temperature above 250° C. being generally suitable. It is frequently advisable to commence with lower temperatures and subsequently to work with higher temperatures. The choice of the added oil depends on the temperature employed, but one and the same initial material may be treated at different temperatures with different added oils, but the oils employed at higher temperatures should preferably be more stable.

The operation is conducted under a pressure of at least 10 atmospheres, very high pressure, as for example above 50 atmospheres and even above 100 atmospheres being preferred. Far higher pressures, for example 1000 atmospheres and more, may also be employed and it may be advisable to operate with different stages of pressure, as for example low pressure during the first stage and then higher pressure during later stages. But in cases where the extraction treatment is followed by a further decomposition treatment, such as cracking or destructive hydrogenation, the process may be conducted at pressures of down to 10 atmospheres. The choice of the pressure depends, inter alia, on the temperature selected, which in turn depends on the character of the initial materials and the added oils.

The result obtained by operating in this manner is that, in contrast to low temperature carbonization, the formation of gases, especially gases which are difficult to condense, is greatly reduced and the yield of liquid products, or products which become liq-

uid when warm, is a multiple of that obtainable by ordinary low-temperature carbonization. The small quantities of gas liberated originate mainly from the substances existing, in an occluded condition, in the materials.

For example, if bituminous brown coal be employed as the initial material, the yield of liquid products, or products which become liquid when warm, is many times the amount corresponding to the bitumen which can be extracted from the initial material by benzene.

As much as 65 per cent of valuable liquid products may be recovered from coals which are even low in bitumen, and alder wood, for example, may be almost completely converted into liquid products by treatment in conjunction with anthracene oil.

The process herein described may be carried out in a continuous manner, for example by mixing the initial material into a paste with the added oil, forcing it by means of pumps through high pressure vessels provided with stirrers, and then releasing the pressure. The stirring may also be effected by means of gases. Other measures may also be adopted to obtain a high relative movement between the added oils and the solid initial material, as for example by creating fresh reaction surfaces by mechanical reduction, kneading and other like means. The product or mixture may also be injected into the reaction vessel in a finely divided state.

The solid bituminous materials and the liquid hydrocarbons may also be passed, in the form of a paste, at a relatively high linear velocity, through a high pressure coil, to effect a sufficient period of contact between said materials to obtain the desired extraction. It is sometimes advisable to pass the mass several times through the apparatus. The continuous operation may also be carried out by mounting a number of vessels, in series or parallel, through which the added oil is passed, some of them being disconnected for recharging with the solid material, and then connected up again, the added oil being brought into action, as desired, by stirring. At the end of such a battery of vessels, units charged with fresh material are connected up in the same proportion as units at the other end are disconnected. Whereas in the cases before mentioned in which the hydrocarbons and solid bituminous materials are formed into a paste and passed together through the system, it is usual to employ unidirectional flow, it is in this case preferable to employ the counterflow principle, the advantages being that the fresh added oil is brought into contact with initial material which has already been exposed to extensive treatment.

The heat of the resulting products may be advantageously utilized by transmission to

the incoming material. The initial material's may also contain water, the drying of the coal being adapted to be combined with the recovery of oil.

5 The product obtained is removed from the pressure chamber, and may, at the same time, under certain circumstances, be quickly relieved of pressure and cooled. After being subjected if required to a preliminary mechanical treatment such as centrifuging and the like, the liquid products are separated from the solid residues in any known and convenient manner, as for example by low temperature carbonization in the presence of 10 steam or other gases and vapors, if desired, extraction or both, or by other means, with or without the application of pressure.

The product obtained, or components of the same may be subjected to cracking in 20 the presence or absence of water vapor or carbon dioxide or another gas or treatment with hydrogen or gases containing the same, with or without the application of pressure, and if desired, with catalysts. In this way, 25 products are obtained of the nature of heavy oils, middle oils, and light oils or benzines. The residual coal is of very loose texture, is easily ignited and readily adsorbs gases. It can be transformed into liquid products 30 by treatment with hydrogen under pressure.

The products obtained by means of the process according to the present invention from an earlier charge may be employed either as they are or after further treatment 35 for application as triturating media for the solid carbonaceous material in the present process, as lubricating oil, Diesel oil or engine fuel and the like, either alone or in admixture with other substances.

40 In carrying out the process it is advisable to see that the material of the apparatus is free from substances which may induce the formation of coke or troublesome viscous masses. For example, it is advisable that 45 finely divided, or porous, iron and nickel, should not be present in such hot portions of the apparatus, especially those parts heated to above 300° C. which come into contact with the substances under treatment. The

50 invention will be further illustrated with reference to the accompanying drawing in which a plant for carrying out the process according to the present invention is illustrated diagrammatically, partly in vertical 55 cross section, although the invention is not limited thereto. *a* is a hopper through which finely divided solid carbonaceous materials can be introduced into a mixing vessel *p*;

*b* is a pipe for the introduction of solvent 60 hydrocarbons into the said vessel *p*. *c* is a stirrer which is actuated by rotation of the wheel *o* the rotation being transferred by means of the tooth gear *m* to the shaft *n*. *d* is a pipe for the transference of the liquid 65 mixtures prepared in the vessel *p* to the

pressure resistant coil *f* which is constructed of alloy steel. *e* is a pump assisting the said transference. *g* is a cooler for cooling the products issuing from the coil *f*. *i* is a pressure release valve for releasing the pressure 70 on the said products. *h* is a settling tank from which the liquid products can be removed by means of the pipe *k*, whereas the solid mixtures are removed by means of the pipe *l*. 75

The following examples will further illustrate how the said invention may be carried into practical effect but the invention is not limited thereto.

#### Example 1

Pulverized brown coal, containing 4 per cent of bitumen which can be extracted by benzene, is made into a paste with an equal amount of anthracene oil containing only a small proportion of constituents boiling below 300°. The mixture is pumped continuously at about 325° C. and under a pressure of 200 atmospheres, through a high pressure vessel, provided with stirring means and constructed internally of highly alloyed steel, a suitable velocity of flow being maintained. After the pressure on the treated coal paste has been relieved, the latter is treated with thinner oil or benzene, or the like, the resulting products being separated from the solid residue. In this way, and practically without any formation of gas, 65 per cent and more of the coal, with reference to ash and water-free initial substance, is transformed into high boiling oils which are liquid at ordinary temperature or when warm. The yield may be further increased by the employment of still higher pressures, for example up to 1000 atmospheres, whereas it becomes considerably smaller if the pressure be substantially reduced, as for example at 20 atmospheres.

Crude brown coal may be replaced, with equal results, by predried brown coal, containing, for example, 10 per cent of moisture, or a brown coal which is substantially richer in bitumen.

The recovered products may be employed, either by themselves or in conjunction with anthracene oil, as trituration media for fresh initial materials, or they may be worked up further into lubricating oil, Diesel oil, engine fuels and the like.

The initial material may also be introduced into the high-pressure chamber through air locks.

#### Example 2

Referring to the accompanying drawing finely divided coal rich in gas is mixed in the vessel *p*, which is fitted with the stirrer *c* with the fractions boiling over 300° C. of a crude mineral oil, both constituents of the mixture being continuously introduced. The paste 120

thus obtained is continuously passed to the compression pump *e* and is forced under a pressure of 200 atmospheres into a pressure-resistant coil *f* constructed of alloy steels 5 which is maintained at a temperature of about 320° C. The products issuing from the said coil are cooled down by means of the cooler *g*. The pressure on the said products is released by means of the valve *i* and 10 they are passed into the separating vessel *h*. The solid materials settling down in the said vessel are drawn off at *l* and the supernatant oil is drawn off through a valve *k*. Any oil floating above the sediment can then be almost 15 completely separated from solid constituents, as for example in a centrifuge. The traces of oil still adhering to the residue can be recovered, for example, by extraction with benzene, and the like, or by steam distillation. More than 55 per cent of the coal is 20 liquefied without any noteworthy production of gas.

*Example 3*

25 An oil shale is continuously treated, at 200 atmospheres pressure and at about 320° C. with a brown coal low temperature tar, which has been freed from constituents boiling below 300° C. 90 per cent and more of the 30 total carbonaceous substance, free from ash and moisture, is obtained in the form of oils.

What we claim is:

1. The process for recovering valuable liquid products from solid bituminous materials which comprises treating said solid materials, in the absence of substantial amounts of hydrogen, with liquid hydrocarbon materials containing substantially no constituents boiling below 300° C. while operating in a 40 system under a pressure of at least 10 atmospheres and a temperature exceeding 250° C. but below the coking temperature of said liquid hydrocarbon materials by continuously passing at least one of said liquid and 45 solid materials through said system and in contact with the other material, contact being effected between said materials until at least 55% of the weight of said solid materials is extracted, introducing additional 50 amounts of said solid and liquid materials into said system and continuously withdrawing the extract from said system.

2. The process for recovering valuable liquid products from solid bituminous materials which comprises treating said solid materials, in the absence of substantial amounts of hydrogen, with liquid hydrocarbon materials containing substantially no constituents boiling below 300° C. while operating in a 60 system under a pressure of at least 50 atmospheres and a temperature exceeding 250° C. but below the coking temperature of said liquid hydrocarbon materials by continuously passing at least one of said liquid and solid 65 materials through said system and in contact

with the other material, contact being effected between said materials until at least 55% of the weight of said solid materials is extracted, introducing additional amounts of said solid and liquid materials into said system and continuously withdrawing the extract from said system. 70

3. The process for recovering valuable liquid products from solid bituminous materials which comprises treating said solid materials, in the absence of substantial amounts of hydrogen, with liquid hydrocarbon materials containing substantially no constituents boiling below 300° C. while operating in a system under a pressure of at 80 least 50 atmospheres and a temperature ranging from 250 to 325° C. by continuously passing at least one of said liquid and solid materials through said system and in contact with the other material, contact being effected between said materials until at least 55% of the weight of said solid materials is extracted, introducing additional amounts of said solid and liquid materials into said system and continuously withdrawing the 85 extract from said system.

4. The process as defined in claim 3 wherein the extraction is effected in the presence of an indifferent gas not giving rise to substantial amounts of hydrogen under 95 the conditions of working.

5. The process for recovering valuable liquid products from solid bituminous materials which comprises treating said solid materials, in the absence of substantial 100 amounts of hydrogen, and in the presence of a catalyst comprising a sulfide and having an alkaline reaction, with liquid hydrocarbon materials containing substantially no constituents boiling below 300° C. while operating in a system under a pressure of at least 50 atmospheres and a temperature ranging from 250 to 325° C. by continuously passing at least one of said liquid and solid materials through said system and in contact 110 with the other material, contact being effected between said materials until at least 55% of the weight of said solid materials is extracted, introducing additional amounts of said solid and liquid materials into said system and continuously withdrawing the 115 extract from said system.

6. The process as defined in claim 5 wherein said catalyst is selected from the class consisting of the alkali metal and alkaline 120 earth metal sulfides.

7. The process for obtaining valuable liquid products from solid bituminous materials which comprises forming a paste of brown coal and anthracene oil containing substantially no constituents boiling below 300° C. passing said paste in the absence of substantial amounts of hydrogen, in a continuous stream through a coil maintained under a pressure of about 200 atmospheres and a tem- 125

perature of about 325° C., the coal and oil remaining in contact in said coil until an extraction of at least 65% of the coal is obtained, continuously removing the products 5 of the extraction from the coil and continuously feeding additional paste into said coil.

In testimony whereof we have hereunto set our hands.

10

KARL WINKLER.  
KURT WISSEL.

15

20

25

30

35

40

45

50

55

60

65